



US006010789A

# United States Patent [19]

Alston et al.

[11] Patent Number: 6,010,789

[45] Date of Patent: Jan. 4, 2000

## [54] POLYESTER STAPLE FIBER

[75] Inventors: **Peter Van Alston**, Kinston; **Patrick Joseph Duncan**; **Steven Michael Hansen**, both of Wilmington, all of N.C.

[73] Assignee: **E. I. du Pont de Nemours and Company**, Wilmington, Del.

[21] Appl. No.: 08/850,457

[22] Filed: May 5, 1997

[51] Int. Cl.<sup>7</sup> ..... C08G 63/68; D02G 3/00

[52] U.S. Cl. ..... 428/397; 428/401; 428/357

[58] Field of Search ..... 428/397, 401, 428/357

## [56] References Cited

## U.S. PATENT DOCUMENTS

5,817,740 10/1998 Anserson et al. ..... 528/295

Primary Examiner—Richard Weisberger

## [57] ABSTRACT

Polyester staple fibers of simple oval peripheral cross-section of aspect ratio at least about 1.85:1 provide advantages both in open-end spinning (to provide yarns with fewer spinning failures than such fibers of conventional round cross-section) and better dye yield in fabrics than polyester staple fibers having other oval cross-sections, especially those having lower aspect ratios.

1 Claim, 1 Drawing Sheet



FIG. 1



## POLYESTER STAPLE FIBER

## FIELD OF INVENTION

This invention relates to improvement in polyester staple fiber, and is more particularly concerned with providing new polyester staple fibers that have an improved cross-section in that the periphery of the new cross-section is a simple oval contour that provides a combination of advantages in open-end spinning and in improved dye yield, and in new spun yarns prepared by open-end spinning such new fibers, and in downstream products of such fibers and yarns, and in processes for obtaining such fibers, yarns and downstream products.

## BACKGROUND OF THE INVENTION

All synthetic fibers, including polyester fibers, can be classified into two groups, namely (1) continuous filaments and (2) fibers that are discontinuous, which latter are often referred to as staple fibers or cut fibers. This invention provides improvements relating to the latter group. Such polyester staple fibers have first been formed by extrusion into continuous polyester filaments, which are processed in the form of a tow of continuous polyester filaments, before the filamentary tow is converted into staple, which is then spun into spun textile yarn, often from blends of polyester fiber with other fibers, mostly cotton fibers or other natural and/or synthetic fibers.

Spinning such staple fibers (which are discontinuous) into continuous yarns or threads, which are generally referred to as "spun yarns" to distinguish them from continuous filament yarns, is one of the oldest processes known to human beings, for instance the use of a spinning wheel. Earlier in the present century, the process generally used commercially was "ring spinning". More recently, however, ring spinning is being mostly replaced by other methods, primarily "open-end spinning", sometimes referred to as "rotor spinning", and by air jet spinning. Aspects of the open-end spinning process, improvements in which are provided by the present invention, have been discussed and described in numerous publications over the last three decades, including, for example, Yngve et al. U.S. Pat. No. 4,729,214, which describes a specific improvement in a particular type of open-end spinning technique, and Ulku et al, in Textile Research Journal 65(10), 557-563 (1995), which discusses the effects of opening roller speed on various different types of fibers in open-end spinning. So far as we know, however, little has been published in the art about the effects on open-end spinning of using fibers of different cross-section.

Open-end spinning is sometimes referred to as OES herein. OES provides a different softer yarn structure than that obtained by air jet spinning. The consequently softer aesthetics of OES yarns are preferred for many end-uses, air-jet yarns having harsher aesthetics because of their different formation and their resulting different yarn structure. The pilling performance of the two yarn structures also differ.

Virtually all polyester staple fibers used to make commercial yarns for the apparel market (except for those in some selected specialty applications) have been of round cross-section for practical and economic reasons. The cross-sectional shape is established by the fiber producer primarily during melt-spinning and is then essentially fixed during drawing and annealing steps used to strengthen the fiber and to stabilize the fine structure of the polyester. Once established by the fiber producer, the cross-section of staple fiber generally remains essentially unchanged during subsequent

mill processing steps used to form the yarns, fabrics and garments. Increasing the complexity of the cross-sectional shape (i.e., making and using any cross-section other than round) has generally increased processing difficulty and costs for fiber producers and especially for fiber processors.

5 Fiber producers prefer to manufacture round fibers over non-round fibers because melt-spinning (extruding) round filaments is most efficient and economical. Round orifices can be easily and economically fabricated. Further, melt-  
10 spinning processes used for round filaments are less demanding than for non-round filaments in that filament formation requires less strict control of polymer viscosity and air quenching to achieve acceptable quality. Immediately after extrusion, the melt tends to swell and form a bulge  
15 under the capillary orifice. Additionally, the uniform and symmetrical surface of the round shape minimizes directional influences during the filament-forming operation and maximizes the opportunity for increasing uniformity of fiber tensile, crimp and lubrication properties, uniformity generally being highly desirable.

20 Likewise, textile processors have preferred to process round fibers over non-round fibers in their normal processing operations because round fibers are easier and more cost-efficient to transform into spun yarns and fabric. This  
25 has been the case particularly in the textile operations of carding, drafting and spinning used to transform the raw cut polyester staple fiber into spun textile yarn. No doubt this has resulted partly from the better property uniformity as discussed above and partly from the uniform friction and  
30 processing characteristics of the symmetrical round surface.

35 Round fibers have also been highly desirable for their economic dyeability and coloring characteristics. Of all potential cross-sections, round fibers possess minimum surface area to color and, therefore, require less dyestuff for  
40 coloration, in contrast to any non-round cross section which must necessarily have increased surface area, so must dye with lower yield and, therefore, generally requires a higher level of costly dyestuffs to achieve the same coloration as a round cross-section.

45 As indicated, both fiber producers and textile mill operators have been driven by economic considerations, so polyester fibers with non-round cross-sections have found little to no use in high volume commodity polyester/cotton blend applications for the commodity apparel market. The few  
50 examples of non-round fibers in the apparel market have been limited to specialty fibers that have provided marketable visual and/or performance fabric and garment attributes that have commanded point of sales premiums to off-set the necessary added producer and textile mill costs.

55 This invention, in contrast, provides a commodity polyester fiber of non-round cross-section that provides, surprisingly, a combination of advantages, namely improved open-end spinning performance over round fibers as well as dye yields equivalent or near equivalent to round fibers, as will be explained hereinafter.

## SUMMARY OF THE INVENTION

According to one aspect, the present invention provides  
60 an improvement in polyester staple fiber having a finish for open-end spinning, said polyester being ethylene terephthalate polymer of relative viscosity 14 to 24 LRV, and said fiber being of 0.4 to 1.5 denier per filament (0.5 to 1.7 dtex) and 25 to 50 mm cut length, said improvement comprising  
65 said fiber having a simple oval cross-section of aspect ratio about 1.85:1 to about 3.5:1. "Simple" oval cross-section is discussed and distinguished from a more complex oval

cross-sectional shape hereinafter. Preferably, the aspect ratio is at least about 2.0:1, especially about 2.25–2.3:1.

We have found that fibers according to the invention have provided efficiency gains in open-end spinning as compared with conventional fibers of round cross-section, by reducing spinning interruptions at fixed processing speeds, or by allowing processing speeds to be increased without exceeding normal mill accepted interruption level with a consequent gain in mill productivity.

Additionally, we have found that the polyester fibers of the invention can be dyed with little or no loss in coloration (i.e., dye yield) using the same weight percent of dyestuff as the commodity round fibers. In contrast, fibers with other oval cross-sections dye significantly lighter than round fibers when the same amount of dyestuff is provided for such fibers, as will be discussed hereinafter.

Also provided according to another aspect of the invention are open-end spun yarns of polyester staple fiber of 0.4 to 1.5 denier per filament (0.5 to 1.7 dtex) and 25 to 50 mm cut length and having a simple oval cross-section of aspect ratio from about 1.85:1, and preferably at least about 2.0:1, to about 3.5:1, said polyester being ethylene terephthalate polymer of relative viscosity 14 to 24 LRV, either alone or mixed with cotton.

According to a further aspect of the invention, there is provided a process of open-end spinning polyester staple fiber alone, or mixed with cotton, said polyester fiber being of 0.4 to 1.5 denier (0.5 to 1.7 dtex) and 25 to 50 mm cut length and having a simple oval cross-section of aspect ratio about 1.85:1, and preferably at least about 2.0:1, to about 3.5:1, said polyester being ethylene terephthalate polymer of relative viscosity 14 to 24 LRV.

Also provided according to the invention are fabrics and garments of such open-end spun yarns.

#### BRIEF DESCRIPTION OF DRAWINGS

FIG. 1 compares the Dye Yield ( $\Delta E$ ) values of dyed fabrics tested of spun yarns of several polyester fibers having different cross-sections vs. the aspect ratios of the various cross-sections, as will be discussed in greater detail hereinafter.

#### DETAILED DESCRIPTION OF PREFERRED EMBODIMENTS

Much of the technology of preparing polyester staple fiber and processing it for spinning into spun yarns by open-end spinning (OES) has been described in the art, so it would be redundant to repeat such disclosure herein.

As indicated, the polyester polymer should be ethylene terephthalate polymer of 14 to 24 relative viscosity (LRV). The polymer may be modified, e.g., with polyethylene oxide (PEO) of molecular weight about 200–2000, in amount about 1 to 5% by weight, to enhance fiber dye rates. Polymer preparation may also include the use of a trifunctional or tetrafunctional chain brancher in amount up to about 0.5 mole %, especially up to about 0.35 mole %, to enhance melt-viscosity as necessary to achieve the desired cross-section shape definition.

The polymer preferably includes a delusterant and/or optical brighteners to screen the normal discolorations associated with polymer manufacture, especially when polymer modifiers are employed, e.g., about 0.1 to about 0.4% by weight of titanium dioxide.

Polyethylene terephthalate containing polyethylene glycol has already been disclosed in the art, e.g., by Snyder in

U.S. Pat. No. 2,744,087 and by De Martino in U.S. Pat. No. 4,666,454, the disclosures of which are hereby incorporated herein by reference. Similarly, the disclosures of Vail U.S. Pat. No. 3,816,486, and Hancock et al., U.S. Pat. No. 4,704,329 are both hereby incorporated herein by reference to disclose examples of processing techniques for preparing drawn annealed fibers and various polymers, and of polymer compositions that may be produced and used according to this invention. Use of copolyester compositions may require adjustment of viscosity appropriately, as described in the art. Finishes suitable for open-end spinning are used commercially and known to those in the art.

Fibers are generally of 0.9 to 1.5 dpf (1 to 1.7 dtex) and are generally cut to staple lengths of 32–38 mm to be suitable for open-end spinning, but may be from 1 inch (25 mm) to 2 inches (50 mm) and are preferably at least 1.25 inches (30 mm) and preferably up to 40 mm cut length. Several people in the trade have shown interest recently in the potential for lower dpf fibers, as indicated, e.g., by Anderson et al in U.S. Pat. Nos. 5,219,506 and 5,219,582, which disclose lower dpf fibers of as low as 0.5 dtex (0.4 dpf), so there is a potential for such lower dpf fibers as feed fibers for OES, as well as for feed fibers that are of more conventional dpf. Mixed deniers, and/or mixed cross-sections including those of the invention with round fibers and other combinations may be used, if desired and advantageous.

An essential feature of the polyester staple fibers according to the invention is their cross-sectional peripheral shape which should be a simple oval of aspect ratio from about 1.85:1, preferably at least about 2.0:1, to about 3.5:1. We use the term "simple oval" herein to distinguish from more complex cross-sections such as, for example, those with deep grooves or indentations or scallops as are disclosed by Gorrafa in U.S. Pat. No. 3,914,488, Franklin in U.S. Pat. No. 4,634,625, Clark et al in U.S. Pat. No. 4,707,407, by Aneja in U.S. Pat. No. 5,591,523, and in application Ser. No. 08/642,650 (DP-6365-A) now allowed, application Ser. No. 08/662,804 (DP-6400) filed Jun. 12, 1996, and by Roop in application Ser. No. 08/778,462 (DP-6550) filed Jan. 3, 1997. The dye yield of polyester staple fiber of scalloped-oval cross-section such as was disclosed, for example, by Gorrafa has been compared with polyester staple fiber according to the invention and the results are included in Example 1 hereinafter, the Gorrafa cross-section being referred to as "4gSO" in Table 1 (for 4 groove scalloped-oval) and its dye yield being 6 shades light, as compared to less than 1 and only 2 shades light for the staple fibers of the invention. Although such scalloped-oval cross-sections are not desirable according to the invention, and a smooth oval cross-section is preferred, as its periphery is not much longer than that of a round cross-section, as will be understood, minor variations from a smooth oval periphery may not significantly increase the dye required and may provide improved OES capability over round fibers.

Also compared in several of the Examples hereinafter vs. polyester staple fiber according to the invention were polyester staple fiber of "Peanut" cross-section, this term for a filament cross-section having been used, for example, in Japanese Patent Application Publication (Kokai), No.: Heisei 4-370,209 (Tanaka Kikinzoku KKK), published Dec. 22, 1992, and being self-explanatory and indicating a peripheral cross-section that has a significant neck halfway along the major axis, instead of having its maximum width at where the minor axis of a simple oval would be located, so not being a simple oval.

Japanese Patent Application Publication Kokai Hei 4-119118 described a polyester fiber with "oval and

deformed cross-section" that was not a simple oval; it did not describe OES, but mostly described use as filament yarns, adding that its fiber could be "of filament or flocculent type"; it referred to several earlier Japanese published applications with various cross-sections that did not, apparently, disclose OES using polyester staple fiber having a simple oval cross-section.

Surprisingly, there has been little discussion of polyester continuous filaments or staple fiber having a simple oval cross-section in the prior art. Johns U.S. Pat. No. 4,410,579 claimed apertured nonwoven fabric of hydraulically-entangled polyester fibers of ribbon-shaped cross-section whose aspect ratio was in the range of 1.8:1 to 3:1, an advantage of such fabrics being their improved disentanglement resistance (see, e.g., col 1, lines 48-52 and FIG. 1). Johns generally used the term "ribbon-shaped" without illustration or further elaboration, but stated that the term meant generally rectangular or oval in shape (col 2, lines 29-30). Johns did not teach open-end spinning, nor indeed any other type of yarn spinning with the staple fiber she used only for hydraulic entangling to form nonwoven fabrics directly from her staple fiber. Chantry et al, U.S. Pat. No. 5,223,187 claimed a continuous process of preparing a high strength monofilament of denier 1,000-10,000 from polyester of very high intrinsic viscosity, such heavy denier monofilaments preferably being of oblong cross-section, with width-thickness ratio greater than 2.0 (col 4, lines 6-12), for use in reinforcing tires. Similarly, Henning, GB 2 221 186 A, disclosed high strength nylon monofilaments of high denier from high viscosity polyamide, desirably of ob-round cross-section, i.e., a generally flat, ribbon-like cross-section with rounded corners (top of page 6). Other disclosures of nylon filaments are Cornelis U.S. Pat. No. 4,012,557, disclosing treating nylon-6 in powder form with aqueous KBr or NaBr and extruding it to form a filament of oval cross-section (e.g., col 4, lines 8, et seq), the dimensions of the resulting filament not being disclosed by Cornelis, and Jennings in U.S. Pat. Nos. 4,702,875 and 4,801,503, disclosing and illustrating (FIG. 2) high tenacity nylon filaments having a ribbon cross-section of length to width ratio greater than 3.

Aspect ratio is the ratio of the major axis to the minor axis of the peripheral cross-section of the polyester staple fiber. As may be seen from the comparative data in Example 1 (Table I), low aspect ratios of 1.5:1 and 1.7:1 for Comparisons D and E would not provide as much advantage as we have obtained by use of staple fiber according to the invention, having cross-sections with higher aspect ratios of about 1.85:1 or more, because Comparisons D and E dyed significantly lighter in shade and so would require significantly more dyestuff; this is also referred to later herein, in relation to FIG. 1. We prefer to use staple fiber of simple oval cross-section having aspect ratios of up to about 3:1. As the aspect ratio increases, there is a tendency towards "glitter", so an aspect ratio of more than about 3.5:1 is generally not desirable, and the desire to avoid "glitter" is one reason why ribbon-shaped cross-sections are not desirable, such ribbon-shaped cross-sections having been mentioned in the art referred to hereinabove.

This invention is further illustrated in the following Examples. All parts, proportions and percentages are by weight unless otherwise indicated.

In each Example, sample filaments of different oval cross-sections were melt-spun from the same polymer recipe and polymer viscosity through different capillaries to give the desired cross-sectional shapes for comparison in open-end spinning and dye yield. Also for comparison, to serve as

a control, i.e., to show the state of the current commercial art as to open-end performance and dye yield, round filaments were spun in the same manner as the test items.

The polymer melt-spun into filaments in each Example 5 was poly(ethylene terephthalate) polymerized with the addition of 0.12 mole % of trimellitate chain-branched (added as trihydroxyethyl trimellitate). As indicated, the polymer in Example 4 also contained a significant amount of PEO. The relative viscosities of the polymers were measured essentially as described by Hancock et al. U.S. Pat. No. 4,704,329, col. 9 lines 6-11, but on a solution obtained by dissolving 0.40 grams of fiber in 5.0 ml. of solvent. The round filaments spun to provide controls were of course spun through circular orifices. The scalloped-oval (4gSO) and peanut 10 filaments spun to provide comparisons were spun through orifices of configuration essentially as shown in FIG. 2 of Clark et al U.S. Pat. No. 4,707,407, and FIG. 6 of Tanaka Japanese Heisei 4-370,209, respectively, both referred to hereinabove. The simple oval comparison filaments D & E in Table I (aspect ratios, respectively, only 1.5:1 and 1.7:1) 15 were spun through orifices shaped like slots, of lengths, respectively, 15 mil (0.38 mm) and 16 mil (0.4 mm), with rounded bulges outwards in the middle of each longer side of the slots, of maximum width, respectively, 7 mil (0.18 mm) and 5 mil (0.15 mm), the slot for D being otherwise shaped like a rectangle with squared corners at each end, while the slot for E had radiused ends. The simple oval 20 filaments spun to provide staple fiber according to the invention (drawn fiber aspect ratios 2.5, 2.7 and 3.2) were all spun through slots with parallel longer sides of overall lengths, respectively, 16 mil (0.4 mm), 15 mil (0.38 mm) and 28 mil (0.71 mm), and widths, respectively, 3.5 mil (0.089 mm), 3 mil 0.076 mm) and 4.3 mil (0.109 mm), the first and third of such slots having radiused ends, while the second 25 was a rectangularly-shaped orifice. As will be understood, these slots produced filaments of simple oval cross-section because the freshly-extruded melt bulged immediately under the orifices, the viscosity of the polymer, the quenching and the wind-up speed being important factors and empirical 30 experimentation generally being desirable to obtain the particular non-round cross-sectional configuration desired, as is understood by those skilled in this art. Oval filaments 35 may be made from orifices of other shapes, as is also well understood, e.g., from orifices that are themselves of oval shape, or with bulges, if desired. The ability to make polyester filaments of various smooth non-round cross-sections was previously known and is not part of the present invention, which is directed to the surprising advantages that 40 we have found in using polyester staple fiber of novel 45 peripheral cross-section as feed fiber for open-end spinning.

The resulting filaments were then drawn, annealed, crimped and lubricated as described to give dpf, tensile and crimp properties as near alike as possible.

Aspect ratio with regards to this disclosure is defined as 55 the ratio of the maximum length to maximum width of the periphery of the filament cross-section, the length being the longest axis, and the length and width axes being perpendicular, normally but not necessarily taken through the centers of the samples. Aspect ratios were obtained by 60 measuring the lengths and widths of multiple samples of drawn fibers, using cross-section images of each particular sample, according to the following procedure. A fiber specimen is mounted in a Hardy microtome (Hardy, U.S. Department of Agriculture circa 378, 1933) and divided into thin sections according to methods essentially as disclosed in "Fiber Microscopy Its Technique and Applications", by J. L. 65 Sloves (van Nostrand Co., Inc., New York 1958, No.

180-182). Thin sections are then mounted on a super FIBERQUANT video microscope system stage (Vashaw Scientific Co., 3597 Parkway Lane, Suite 100, Norcross, Ga. 30092) and displayed on the Super FIBERQUANT CRT under magnifications as needed. The image of an individual thin section of one fiber is selected and critical fiber dimensions measured. The ratios are then calculated. This process is repeated for each filament in the field of view to generate a statistically significant sample set, and the averages are given herein.

Tensile properties were measured using either a Model 1122 or 1123 Instron on fibers cut to 0.5 inch (13 mm) sample lengths.

Finish levels are given as FOT % (Finish on Tow) and were obtained on polyester fiber cut from the tow, using the well known tube elution method that gravimetrically determines the weight percent of finish oils after extracting the oils from the fiber with methanol, as a percentage of the weight of the fiber.

CPI (crimps per inch) were determined conventionally by counting the number of crimps per extended length of filament.

Open-end spinning (OES) trials were carried out on Schlafhorst SE-9 or SE-8 spinning frames using 100% or 50/50 cotton blend sliver prepared as described in the Examples. Spinning frame setup and conditions (including room temperature—humidity conditions) were held constant during each Example except for any adjustment of rotor speed per test design. For each Example, items were assayed one by one over a common set of 24 machine positions (rotors) for periods of 5 to 10 hours. Ends down (yarn formation failures in the spinning box) were tracked by the SE-8 or SE-9 instrumentation and the failure data normalized to express failures in terms of 1000 rotor hours for each item.

## EXAMPLES

### Example 1

Polyester filament samples having different oval-shaped cross-sections were melt-spun from polymer of 19 LRV through spinnerets fitted with capillaries designed to give different specific cross-section shapes in the fully-drawn fibers. Filaments were collected at 1800 yards per minute (1650 ppm) on bobbins using a commercial winding device. Bobbin lots of 2.5 and 3.2 aspect ratio simple oval cross-section according to the invention were prepared in this manner as well as the following comparisons that are not according to the invention, namely simple oval cross-sections of lower aspect ratio 1.5 and 1.7, more complex peanut-shaped and a 4 groove (4gSO) scalloped-oval cross-section, and a round cross-section as a control. Each bobbin lot was combined into a tow (from a creel) which was drawn, steam-annealed, crimped and dried to give a denier per filament of 1.2 (1.3 dtex) and similar tensile and crimp properties as given in Table 1. The same standard commercial lubrication useful for open-end spinning was applied to all the items during the drawing and crimping operation. The tensile and crimp properties and finish (FOT) in Table 1 are for the raw fibers.

Each test lot was cut to standard 1.25 inch (32 mm) fiber length, carded as 100% polyester and draw frame blended with 70 grain (4.5 gm) carded cotton to give a 50/50 polyester cotton blend sliver of 68 grain (4.4 gm) weight. Finisher drawing completed the draw blending operation and reduced the sliver weight to 60 grains (3.9 gm).

The slivers indicated were competitively spun into 28/1 cc (210 dtex) yarns on common rotors of a Schlafhorst SE-9

against the round control and the results are shown in Table 1, from which it can be seen that all the oval shapes tested gave significant reductions in ends down, i.e., significant improvements in OES process capability over the round commercial control.

Additionally, each item was spun into 100% 20/1 cc (295 dtex) open-end yarns on a Schlafhorst SE-8. The resulting yarns were knitted into fabrics and then dyed in separate baths using 2% Terasil Blue GLF dyestuff per gram of fabric and a dye bath rate of rise of 3° F. (2° C.) per minute from room temperature up to 260° F. (127° C.) with a 30 minute hold at 260° F., a typical procedure used commercially for the dyeing of polyester. The dyed fabrics were then dried and instrumentally compared on a Color Mate HDS Color Analyzer using D65 standard daylight illuminant. The instrument provides a Delta E value that quantifies any difference from the color of the round fiber standard. A Delta E value greater than 0.7 units from standard is estimated as a dye shade difference of 1, so, for convenience, the number of shade differences are shown in Table 1 as well as the Delta E values.

The dye advantage for simple oval cross-sections according to the invention is easily seen from Table 1, in contrast to oval cross-sections having Aspect Ratios of 1.5 and 1.7, which incurred substantial dye yield losses of 3 and 7 shades. Likewise, 4.5 and 6 shades of dye yield loss were incurred with the more complex cross-sections such as the peanut and the 4 g scalloped-oval cross-section, although the peanut cross-section had an aspect ratio within the range of 2 to 3.5.

In other words, polyester staple fibers according to the invention having simple oval cross-sections with high enough aspect ratios showed significant improvements in OES process capability (at most about half the number of ends down as tested and compared with the round standard) without much dye yield loss as compared with the same commercial standard, and in contrast to the other cross-sections tested, which showed significant dye yield losses.

TABLE 1

|    | CON-                            | COMPARISONS  |              |              |              |              | IN-          |              |
|----|---------------------------------|--------------|--------------|--------------|--------------|--------------|--------------|--------------|
|    |                                 | A            | B            | C            | D            | E            | VENTION      |              |
|    |                                 |              |              |              |              |              | 1            | 2            |
| 45 | Fiber Shape                     | round        | 4gSO         | peanut       | oval         | oval         | oval         | oval         |
|    | Aspect Ratio                    | 1.0          | 1.6          | 2.2          | 1.5          | 1.7          | 2.5          | 3.2          |
|    | Fiber Properties                |              |              |              |              |              |              |              |
| 50 | Tenacity g/d<br>(g/dtex)        | 5.2<br>(4.7) | 5.2<br>(4.7) | 5.3<br>(4.8) | 5.0<br>(4.5) | 5.1<br>(4.6) | 4.9<br>(4.4) | 5.3<br>(4.8) |
|    | T <sub>10</sub> g/d<br>(g/dtex) | 4.1<br>(3.7) | 3.8<br>(3.4) | 4.0<br>(3.6) | 3.5<br>(3.2) | 3.9<br>(3.5) | 3.8<br>(3.4) | 3.8<br>(3.4) |
|    | Elongation, %                   | 20           | 19           | 19           | 24           | 22           | 18           | 18           |
|    | CPI<br>(CPem)                   | 9.2<br>(3.6) | 8.7<br>(3.4) | 9.4<br>(3.7) | 8.7<br>(3.4) | 9.5<br>(3.7) | 7.9<br>(3.1) | 9.5<br>(3.7) |
|    | FOT %                           | 0.16         | 0.17         | 0.17         | 0.15         | 0.14         | 0.17         | 0.15         |
| 55 | OES Process<br>Capability       |              |              |              |              |              |              |              |
|    | Ends Down/1M                    | 303          | —            | —            | 60           | 72           | 153          | 119          |
|    | Rotor Hours - at<br>105M RPM    |              |              |              |              |              |              |              |
|    | Dye Yield<br>Properties         |              |              |              |              |              |              |              |
| 60 | Delta E<br>Shades Light         | std          | 4.3          | 3.3          | 5.0          | 2.2          | 0.6          | 1.4          |
|    |                                 | std          | 8            | 4.5          | 7            | 3            | <1           | 2            |

### Example 2

Another set of filaments having different cross-sections were prepared essentially as described in Example 1. These

bobbin lots had fibers having a normal round cross-section as a control, a simple oval of 2.7 aspect ratio according to the invention, and two peanut cross-sections, each of aspect ratio 2.0 as comparisons. Their properties are listed in Table 2.

These items were cut to a standard 1.25 inch (32 mm) length and then preblended 50/50 with cotton before the blends were carded to 70 grain (4.5 gm) slivers, and then drawn in 2 steps to 60 grain (3.9 gm) slivers for open-end spinning trials, and dye yield comparisons essentially as described for Example 1. The results are given in Table 2 and show the dramatic reductions in ends down for the simple oval cross-section according to the invention, and for the peanut cross-sections, but significant dye yield loss for the peanut cross-sections in contrast to the excellent dyeing performance for the fiber of simple oval cross-section according to this invention. Indeed, this simple oval cross-section according to the invention dyed more deeply than the round control.

TABLE 2

| FIBER PROPERTIES                             | COMPARISONS   |            |            | INVENTION  |
|----------------------------------------------|---------------|------------|------------|------------|
|                                              | Round Control | Peanuts    | Oval       |            |
| Aspect Ratio                                 | 1.0           | 2.0        | 2.0        | 2.7        |
| Tenacity g/d (g/dtex)                        | 5.6 (5.0)     | 5.2 (4.7)  | 4.3 (3.9)  | 4.9 (4.4)  |
| T <sub>10</sub> g/d (g/dtex)                 | 4.3 (3.9)     | 4.3 (3.9)  | 2.7 (2.4)  | 3.5 (3.2)  |
| Elongation, %                                | 18            | 15         | 17         | 17         |
| CPI (CPcm)                                   | 9.7 (3.8)     | 11.0 (4.3) | 10.2 (4.0) | 10.6 (4.2) |
| FOY %                                        | 0.13          | 0.16       | 0.13       | 0.14       |
| <u>OES Process Capability</u>                |               |            |            |            |
| Ends Down/1M Rotor Hours - at 110M RPM Rotor | 735           | 155        | 125        | 275        |
| <u>Dye Yield Capability</u>                  |               |            |            |            |
| Delta E                                      | std           | —          | 3.3        | 0.4*       |
| Shades Light                                 | std           | —          | 5          | 0          |

\*Dyed darker (i.e., better) than the round control standard.

### Example 3

Filaments were spun, drawn and converted into staple essentially as described in Example 1 and then, as 100% polyester staple fiber, were carded to 60 grain (3.9 gm) slivers and drawn in two steps to 50 grain (3.2 gm) slivers and assayed for performance capability on a Schlaufhorst SE-8 open-end frame. The performance data showed that the round cross-section polyester staple gave an unacceptably high level of ends down (420/1000 rotor hours exceeding commercial goal of no more than 200) at 70,000 RPM rotor speed, whereas the polyester fiber of simple oval cross-section according to this invention gave zero ends down at a higher rotor speed of 75,000 RPM. The peanut oval comparison also gave excellent open-end performance, but unacceptable loss in dye yield, in contrast to the fiber of the invention, as indicated in Table 3.

TABLE 3

| FIBER PROPERTIES             | COMPARISONS   |             |             | INVENTION |
|------------------------------|---------------|-------------|-------------|-----------|
|                              | Round Control | Peanut      | Oval        |           |
| Aspect Ratio                 | 1.0           | 2.0         | 2.7         |           |
| Dpf (dtex)                   | 1.05 (1.17)   | 1.05 (1.17) | 1.02 (1.13) |           |
| Tenacity g/d (g/dtex)        | 5.8 (5.2)     | 5.9 (5.3)   | 5.9 (5.3)   |           |
| T <sub>10</sub> g/d (g/dtex) | 3.7 (3.3)     | 4.7 (4.2)   | 4.6 (4.1)   |           |
| Elongation, %                | 16            | 13          | 13          |           |

TABLE 3-continued

| 5                    | FIBER PROPERTIES | COMPARISONS   |            | INVENTION |
|----------------------|------------------|---------------|------------|-----------|
|                      |                  | Round Control | Peanut     |           |
| CPI (CPcm)           | 11.3 (4.4)       | 9.6 (3.8)     | 10.1 (4.0) |           |
| FOT %                | 0.10             | 0.14          | 0.12       |           |
| Dye Yield Capability |                  |               |            |           |
| 10                   | Delta E          | std           | 3.1        | 0.4       |
|                      | Shades Light     | std           | 4          | <1        |

### Example 4

Sample filaments having round cross-section (as a control again) and simple oval cross-section according to the invention were produced from polymer of about 20.3 LRV and about 2.3% by weight of PEO, poly(ethylene oxide) of 600 MW, but in other respects essentially as described in Example 1, and were processed and spun into yarns at a rotor speed of 107,000 RPM and compared also essentially as described in Example 1. Relevant parameters and results are summarized in Table 4, from which it can be seen that the fibers of simple oval cross-section according to the invention were processed into spun yarn much better (only a quarter of the failures encountered with the round control) without much loss in dye yield.

TABLE 4

| 30 | POLYMER                                            | CONTROL          |             | INVENTION |
|----|----------------------------------------------------|------------------|-------------|-----------|
|    |                                                    | LRV              | 20.4        |           |
|    |                                                    | 6000MW PEO, wt % | 2.1         |           |
|    | <u>Fiber Properties</u>                            |                  |             |           |
| 35 | Fiber Cross-section                                | round            | oval        |           |
|    | Aspect Ratio                                       | 1.0              | 2.5         |           |
|    | Denier/Filament (dtex)                             | 1.24 (1.38)      | 1.28 (1.42) |           |
|    | Tenacity gpd (g/dtex)                              | 5.9 (5.3)        | 5.1 (4.6)   |           |
|    | T <sub>10</sub> gpd (g/dtex)                       | 3.7 (3.3)        | 2.2 (2.0)   |           |
|    | Elongation, %                                      | 21               | 21          |           |
|    | CPI (CPcm)                                         | 9.2 (3.6)        | 9.1 (3.6)   |           |
|    | FOT %                                              | 0.14             | 0.15        |           |
|    | <u>OES Process Capability</u>                      |                  |             |           |
| 40 | Ends Down/1M Rotor Hours - at 107M RPM Rotor Speed | 228              | 55          |           |
|    | <u>Dye Yield Capability</u>                        |                  |             |           |
|    | Delta E                                            | std              | 1.0         |           |
|    | Shades Light                                       | std              | 1.5         |           |

For convenience, the Dye Yields (Delta E values) for 50 various fiber cross-sections that we have tested and measured have been plotted vs. the Aspect Ratios of the cross-sections of the constituent polyester staple fibers in the yarns of the dyed fabrics and are shown in FIG. 1 of the accompanying drawings. A round cross-section standard has an 55 Aspect Ratio of 1.0:1 and a ΔE of 0.0. The simple oval cross-sections of various aspect ratios mostly required more dye (except for the oval cross-section of Example 2 that dyed darker than the round control standard) as shown in FIG. 1, and generated a curve, as shown, indicating a 60 relationship between aspect ratio and ΔE, wherein for oval fibers of low aspect ratio (not according to the invention) the ΔE increased very sharply as the aspect ratio was increased from 1.0:1, and then, after peaking, decreased sharply as the aspect ratio was further increased beyond the peak, and then, 65 after dropping below a ΔE value of about 1.0, at an aspect ratio of about 1.85:1, the rate of decrease of the ΔE with increasing aspect ratio levelled off and the curve becomes

quite flat at an aspect ratio of about 2.0:1, and then, after a higher aspect ratio (about 2.5:1), the  $\Delta E$  increases somewhat with increasing aspect ratio. The relationship between  $\Delta E$  and aspect ratio was very surprising. It was especially surprising to find that the  $\Delta E$  for aspect ratios of about 1.85:1 and more were so significantly less than for oval cross-sections of lower aspect ratio, such as 1.5:1, and that such polyester staple fibers gave significant advantages in open-end spinning over conventional polyester staple fiber of round cross-section, but dyed so much more efficiently than polyester staple fiber having other oval cross-sections, especially those of lower aspect ratio. In addition to the plots for simple oval cross-sections, the complex oval cross-sections are shown in FIG. 1 as "x" points, for the (4 groove) scalloped-oval cross-section and the peanut cross-sections used as Comparisons in the foregoing Examples.

As indicated, we have found that the  $\Delta E$  dye yield is about 1.0 or less when the aspect ratio is about 1.85:1 or more, i.e., use of simple oval cross-sections having such aspect ratios, surprisingly, have given shade differences of about 1.5 or less as compared with conventional round cross-sections, together with improved open-end spinning capability. When

the slope of the curve is relatively steep below about 2.0:1, and especially below about 1.9:1 aspect ratio, the dye yield becomes more sensitive to aspect ratio changes, so that dye yield management becomes more difficult. This is one reason why we prefer to operate outside such a potential problem area, i.e., at least about 2.0:1, and especially at about 2.25:1 aspect ratio or more. However, with proper care, e.g., of spinneret design and careful polymer viscosity management, we believe that somebody could operate using lower aspect ratios, such as 1.85-1.95, and get acceptable dye yields.

We claim:

1. Improvement in polyester staple fiber having a finish for open-end spinning, said polyester being ethylene terephthalate polymer of relative viscosity 14 to 24 LRV, and said fiber being of 0.4 to 1.5 denier per filament and 25 to 50 mm cut length, said improvement comprising said fiber having a simple oval cross-section of aspect ratio about 1.85:1 to about 3.5:1.

\* \* \* \* \*